

# UNITED STATES PATENT OFFICE.

JAMES M. ALLEN, OF ST. LOUIS, MISSOURI, ASSIGNOR TO FELLHAUER-ALLEN MANUFACTURING COMPANY, OF ST. LOUIS, MISSOURI, A CORPORATION OF MISSOURI.

## REFRACTORY MATERIAL.

1,275,354.

Specification of Letters Patent. Patented Aug. 13, 1918.

No Drawing.

Application filed November 10, 1917. Serial No. 201,250.

To all whom it may concern:

Be it known that I, JAMES M. ALLEN, a citizen of the United States, and a resident of St. Louis, State of Missouri, have invented a new and useful Refractory Material, of which the following is a specification.

The object of my invention is to produce a comparatively simple and inexpensive refractory material which is particularly applicable for making crucibles, retorts, fire brick and tile, furnace linings and like articles and products which are necessarily subjected to comparative high degrees of heat. 10  
My composition consists of a mixture of two or more varieties of fire clay, a carbonaceous material such as anthracite coal and a mineral cementing and glazing material, such as galena or lead oxid. 15  
In preparing the composition to manufacture my improved refractory material, I prefer to use the ingredients in about the following proportions: pulverized fire clays 48½%, pulverized anthracite coal 48½%, and 20 pulverized galena, or lead oxid 3%.

Satisfactory results may be obtained, however, when the ingredients are varied within the following limits—from 40 to 58 per cent. fire clay, and from 40 to 58 per cent. anthracite coal, the remainder being galena, or lead oxid. 25

These ingredients are thoroughly mixed with each other and with a quantity of water sufficient to form a comparatively stiff paste, 30 which can be readily worked with the hands or molded in suitable forms.

After the articles have been properly formed and air-dried they are subjected to heat from 1,400 to 2,500 degrees Fahrenheit, 35 and the resultant product is very hard, having a glazed or semi-glazed surface, and is refractory to a high degree.

In my improved material I prefer to use two or more different varieties of fire clay in order to form a perfect bond and readily 45 workable material while being mixed. Further, by using two or more varieties of fire clay the finished product has a body which is of the same density throughout its walls or dimensions. The coal in the finished product provides the necessary expansive element and it will be understood that when the product is first subjected to heat, certain volatile gases will be given off from the coal and the resulting ash is bonded to 50 the surrounding clay so that when the material is later subjected to heat it will readily expand and contract as a result of varying 55 temperatures.

The galena or lead oxid materially assists 60 in bonding the clay and coal together and provides the finished material with a comparatively smooth glazed or semi-glazed surface. Refractory material of my improved construction is particularly adapted for use 65 in the formation of crucibles and retorts, and said material can be subjected to great heat without flaking or cracking.

I claim—

1. The herein described refractory material composed of two or more varieties of fire clay, anthracite coal and galena. 70
2. The herein described refractory material comprising from 40 to 58 per cent. fire clay, from 40 to 58 per cent. anthracite coal, 75 and a comparatively small amount of galena.
3. The herein described refractory material consisting of 48½ per cent. fire clay, 48½ per cent. anthracite coal and 3 per cent. galena. 80

In testimony whereof I hereunto affix my signature, this thirtieth day of October, 1917.

JAMES M. ALLEN.